

May 4, 1926.

1,583,573

T. H. BUTLER ET AL

PROCESS FOR THE PRODUCTION OF FUEL MIXTURES

Filed Dec. 21, 1925



*INVENTORS*

Thomas Howard Butler  
Herbert William Patterson  
Eric William Parkes

BY

*Gill and Jennings*  
ATTORNEYS

Patented May 4, 1926.

1,583,573

# UNITED STATES PATENT OFFICE.

THOMAS HOWARD BUTLER, OF BRISTOL, HERBERT WILLIAM ROBINSON, OF CLEOBURY MORTIMER, AND DERICK WILLIAM PARKES, OF BIRMINGHAM, ENGLAND.

## PROCESS FOR THE PRODUCTION OF FUEL MIXTURES.

Application filed December 21, 1925. Serial No. 78,846.

To all whom it may concern:

Be it known that we, THOMAS HOWARD BUTLER, HERBERT WILLIAM ROBINSON, and DERICK WILLIAM PARKES, British subjects, and residents of Bristol, England, Cleobury Mortimer, England, and Birmingham, England, have invented a certain new and useful Improved Process for the Production of Fuel Mixtures, of which the following is a specification.

This invention relates to the production of fuels containing coal tar pitch, and fuel oil of petroleum or asphaltic origin. The fuel value of pitch has been, of course, already recognized and attempts have been made to blend pitch with fuel oils such as petroleum.

When pitch is blended with fuel oil of the above kinds there is a tendency for the bitumen to separate out and to carry with it the free carbon. A process has been devised as set forth in United States Patent No. 1,567,235 dated December 29th, 1925, according to which fuel oil is stirred into pitch which is maintained substantially above its melting point during the process. Such a mixture remains homogeneous as long as it is maintained above certain temperatures. If pitch and fuel oil be mixed in certain proportions which depend upon the kind of fuel oil and also the grade of coal tar pitch, mixtures may be obtained which are homogeneous at all temperatures. It is, however, practically impossible in practice to determine accurately the necessary proportions. It is the object of the present invention to produce a pitch and fuel oil mixture in such a condition that it will remain as a homogeneous mixture at all temperatures with certainty and can, therefore, be used as a liquid fuel, although in some cases it may have to be melted for this purpose.

According to the present invention, a fuel mixture is obtained by distilling coal tar together with fuel oil of petroleum or asphaltic origin. The distillation of such coal tar and petroleum residuum may be carried out with or without the use of steam or vacuum or both. The proportions of the materials taken and the point to which the distillation is carried have no effect on the permanent homogeneity of the mixture obtained. The specific gravity of the creosote fraction of the distillate is usually less than that of

creosote obtained from coal tar in the usual way, but the specific gravity may be raised by increasing the proportion of coal tar in the original mixture to be distilled. Residues from such a distillation process may be of any viscosity, that is to say may vary from the liquid condition to the solid condition depending upon the proportions of the starting materials and the extent to which the distillation is carried. The fact is that the distillation process has the effect of automatically adjusting the ratio of the amounts of the pitch and the fuel oil in the residue to ensure that that ratio is correct to enable the mixture to remain homogeneous at all temperatures. Further, petroleum residuum may be added to such residues but the products obtained are then not homogeneous at all temperatures, but generally speaking, they have a better range of stability than mixtures obtained by mixing coal tar pitch directly with petroleum residuum.

Some embodiments of the present invention will now be described with reference to the accompanying drawing which is a diagrammatic side elevation of an apparatus which may be employed in carrying out the novel process.

In that drawing, A is the still mounted in brickwork B, and heated by means of the furnace C. In carrying out steam distillation, the steam is introduced through the pipe D provided with the control valve E and emerges into the still A by way of the perforated pipe F. The vapours are condensed in the condenser G and flow into the receiver H. A vacuum pump K may be employed when it is desired to carry out the distillation under vacuum.

The following examples of the novel process may be cited. 100 parts by weight of coke oven tar and 50 parts by weight of Mexican fuel oil having a specific gravity of 0.950 and 15 per cent of the fuel oil distilling off up to a temperature of 300 degrees C. are distilled up to a temperature of 370 degrees C. until 50 parts by weight of distillate are obtained. The residue obtained is homogeneous at all temperatures and is liquid below 100 degrees C.

According to another example, 100 parts by weight of the same coke oven tar and 60 parts by weight of the same fuel oil are distilled at 370 degrees C. until 60 parts of the

distillate are taken off. The residue is solid at normal air temperature and has a bright conchoidal fracture. It is liquid below 125 degrees C. and is perfectly homogeneous at all temperatures.

According to yet another example, 500 parts by weight of the same coke oven tar and 125 parts by weight of the same fuel oil are subjected to steam distillation until 260 parts by weight of distillate are taken off. The creosote fraction of the distillate amounts to 0.48 litres per kilogram of the original coke oven tar taken. The residue is homogeneous at all temperatures. The residue may be mixed with a certain amount of fuel oil of the same quality, for example, 71 parts by weight of the residue with 29 parts by weight of the fuel oil. The resulting product is homogeneous down to 150 degrees C., but below this temperature becomes grainy, but no bituminous matter actually separates out.

According to a fourth example, 500 parts by weight of the same coke oven tar and 75 parts by weight of the same fuel oil are subjected to steam distillation until 242 parts of distillate are taken off. In this case the creosote fraction amounts to 0.412 litres per kilogram of the original tar. The residue again is entirely homogeneous at all temperatures. It may be mixed with fuel oil of the same quality in the proportions of 62 parts by weight of the homogeneous mixture to 38 parts by weight of the fuel oil. The product is only homogeneous above 165 degrees C. becoming grainy at that temperature and deposits bituminous matter at 130 degrees C.

According to a final example, 500 parts by weight of the same coke oven tar and 85 parts by weight of the same fuel oil are distilled until 249 parts by weight of the distillate are taken off. The creosote fraction of the distillate in this case amounts to 0.41 litres per kilogram of the original tar. The mixture may be mixed with fuel oil of the same quality in the proportions of 67 parts by weight of the mixture to 33 parts by weight of the fuel oil. The resulting product is only homogeneous above 145 degrees C. at which temperature it becomes grainy and deposits bituminous matter at 110 degrees C.

It will be understood that the above are

merely given as examples of certain proportions of specific materials which may be used to make the fuel mixtures. It will be understood, of course, that the invention is not limited to the particular proportions given in any of the examples for, as already stated, whatever proportions are used the distillation adjusts the conditions so that the mixture is completely homogeneous at all temperatures. It will also be understood that coal tars of other grades may be employed as well as other fuel oils of petroleum or asphaltic origin. Moreover, if additional fuel oil is added to the entirely homogeneous mixture so that the resulting product is only homogeneous above a certain critical temperature, that critical temperature may be reduced by the addition of solid hydrocarbons obtained from the distillation of coal tar such as solid hydrocarbons of the naphthalene or anthracene series.

Having thus described our invention, what we claim as new and desire to secure by Letters Patent is:—

1. A process for obtaining a mixture containing pitch and fuel oil of the character set forth, which consists in distilling the said fuel oil together with coal tar, the residue from such distillation containing the desired mixture.

2. A process for obtaining a fuel mixture containing pitch and petroleum residuum, which consists in distilling the petroleum residuum with coal tar with the use of steam, the residue from such distillation containing the desired mixture.

3. A process for obtaining a fuel mixture containing pitch and petroleum residuum, which consists in distilling the petroleum residuum with coal tar with the use of steam and vacuum, the residue from such distillation containing the desired mixture.

4. A process for obtaining a fuel mixture containing pitch and a fuel oil of the character set forth, which consists in distilling the said fuel oil with coal tar and stirring in further fuel oil to the residue obtained from the distillation.

In witness whereof we hereunto subscribe our names this 23rd day of November, 1925.

THOMAS HOWARD BUTLER.

This 4th day of December 1925.

HERBERT WILLIAM ROBINSON.

DERIC WILLIAM PARKES.